

Jan. 10, 1967

C. J. SPEERSCHNEIDER

3,297,417

BERYLLIUM COATING FOR BERYLLIUM

Filed March 26, 1964

FIG 1



FIG 3



**1**

3,297,417

**BERYLLIDE COATING FOR BERYLLIUM**

Charles J. Speerschneider, Minnetonka, Minn., assignor to  
Honeywell Inc., a corporation of Delaware  
Filed Mar. 26, 1964. Ser. No. 354,904  
8 Claims. (Cl. 29—199)

Generally, this invention is directed to low friction, wear resistant coatings for beryllium. More specifically, this invention is concerned with a beryllide intermetallic coating for beryllium and a method for preparing such coatings.

Beryllium has achieved widespread use due to its low density and relatively high strength. It has found particular application in gas bearing structures as a basic material. However, this use has been quite limited since beryllium has poor resistance to wear and a high coefficient of friction. Consequently, a low friction, wear resistant adherent coating for the beryllium is necessary.

Hard ceramic materials have been used previously as a coating for beryllium to obtain improved resistance to wear over the basic beryllium material. One technique used to obtain such coatings has been the flame spraying of beryllium with materials such as alumina. These coatings result in relatively good resistance to wear, however, they are porous and thus undesirable from a bearing dynamics standpoint. Also, this hard surfacing material is sprayed directly onto the beryllium surface with no transition zone between the relatively soft beryllium and the relatively hard ceramic. A transition zone is desirable since it results in a gradual change in properties reducing the stress concentrations and increasing adhesion. A second technique which has been utilized is an anodizing procedure. However, again porosity is present in addition to processing difficulties in controlling beryllium oxide coatings.

It has been found that surface coatings of gamma-nickel beryllide ( $Ni_5Be_{21}$ ) having substantial thickness can be applied to both flat and cylindrical beryllium surfaces using a diffusion technique. The coatings are very hard, have a high surface density (non-porous) and are adherent to the beryllium base material. Good adhesion is due to the formation of a two phase transition region between the gamma-nickel beryllide and the beryllium. In order to obtain this two phase region a third element, silver, is necessary and is best introduced as an alloying agent in the beryllium.

It is an object of this invention to improve beryllium for use as a bearing material, particularly in gas bearing applications.

It is another object of this invention to provide a low friction, wear resistant coating for beryllium having good adherence due to the presence of a two phase transition region.

It is a further object of this invention to provide a low friction, wear resistant coating for beryllium which has a high surface density, i.e., a non-porous coating.

It is another object to provide a beryllide coating for beryllium having a hardness which is comparable to coatings used in the prior art and which has excellent adherence to the beryllium base material.

It is a still further object of the invention to provide a diffusion bonding method for preparing beryllide coatings on beryllium which results in a coating having superior properties over those of the prior art.

It is another object to provide a diffusion bonding method for preparing beryllide coatings on beryllium in which relatively thick coatings can be prepared in a short time.

It is still another object to provide a method for preparing beryllide coatings on beryllium which results

**2**

in highly adherent coatings due to the formation of a two phase transition region in the coating.

It is a still further object to provide a novel method for preparing beryllide coatings on beryllium which utilizes silver to form a two phase transition region in the coating.

These and other objects and advantages of the present invention will become evident from the following description in which:

FIGURE 1 is a schematic representation of a diffusion couple of nickel and beryllium showing the various regions formed therebetween as a result of heating.

FIGURE 2 is a graph showing the shear strength and fracture path of various diffusion couples.

FIGURE 3 is a graph showing the effect of time, temperature and silver alloy content on total beryllide thickness.

Briefly, the beryllide intermetallic coating prepared in accordance with this invention is composed of two regions (1) gamma-nickel beryllide ( $Ni_5Be_{21}$ ) and (2) a two phase region of gamma-nickel beryllide plus a beryllium-silver alloy ( $Ni_5Be_{21} + Be - Ag$ ). These regions are formed by a diffusion bonding technique. The technique involves the contacting of a beryllium base material by a body of nickel and a subsequent heat treatment. In order to obtain the desired two phase transition region between the nickel beryllide ( $Ni_5Be_{21}$ ) and the beryllium, a third element is necessary. This is silver which may be introduced in various ways as will be discussed hereinbelow. After introduction of the silver, heating forms a diffusion bond between the nickel and beryllium as shown schematically in FIGURE 1. This type of structure is termed a diffusion couple and is composed of five regions;

Region A—nickel  
Region B— $NiBe(\beta)$   
Region C— $Ni_5Be_{21}(\gamma)$   
Region D— $Ni_5Be_{21} + Be - Ag$  (two phase)  
Region E—beryllium or beryllium-silver

Subsequent to the diffusion bonding, regions A and B are removed by grinding or the like to expose the gamma-nickel beryllide of region C thus providing a two layer beryllide coating for the beryllium base material.

**Procedure**

The method used in diffusion bonding begins with the cleaning of the beryllium base material and the nickel material by standard procedures which are well known in the art such as abrading the surfaces with a fine grit. The two bodies are then placed in contact under a light load (sufficient to maintain contact between the work pieces) and heated in a vacuum. For curved surfaces, a molybdenum sleeve with its low coefficient of thermal expansion is used to maintain intimate contact at elevated temperatures whereas a very light, dead weight load is used with diffusion couples of the type shown in FIGURE 1. The applied temperature has been found to be critical in that it must be at least about 1075° C. to obtain bonding through formation of the two phase region. Higher temperatures are limited only by the fact that they should not exceed the melting point of the beryllium. A preferred temperature range has been found to be about 1100° C. and above due to increasing hardness and thickness of the coating produced with increasing temperatures. A heating time of at least 1/2 hour is required to form the desired diffusion region.

**Silver**

As previously stated, the presence of silver is required to obtain the two phase region designated as D in FIGURE 1. The two phase region provides a transition zone

from the relatively soft beryllium to the extremely hard gamma-nickel beryllide ( $Ni_3Be_{21}$ ). A transition zone is necessary since it allows for a gradual change in properties thus reducing stress concentration and increasing adhesion. This is confirmed by the fact that, in diffusion couples prepared in the same way as discussed above, but without added silver, the two phase region was absent and the couples separated during handling.

The silver may be introduced into the diffusion couple in many ways. Plating either the nickel or beryllium with silver or inserting a thin sheet of silver between the two bodies prior to heating has been found to produce the desired results. A silver plate formed on the nickel body which is then placed in contact with the beryllium and bonded has been found to be particularly satisfactory. The amount of the silver plate entering into the reaction is determined by the temperature to which the couple is heated since the solubility of the silver is dependent on temperature.

An alternate approach for including the silver is to incorporate it directly into the beryllium base material. This is accomplished by standard powder metallurgy techniques. The most satisfactory results have been obtained when an alloy has been used consisting of 1-8% silver, balance beryllium.

#### Adherence

A measure of the shear strength of sample beryllium-nickel diffusion couples shows that strength varies with alloy addition from 6000 p.s.i. for beryllium-8% silver to 2800 p.s.i. for beryllium-1% silver. FIGURE 2 shows how the shear strength of the beryllium-nickel diffusion couples varies with silver additions from 6000 p.s.i. for beryllium-8% silver and silver plated nickel (excessive silver) to 2800 p.s.i. for beryllium-1% silver. More important, an examination of the fracture path in the various samples as noted in FIGURE 2 shows that for the beryllium-8% silver alloy, fracture occurs either within the gamma-beryllide layer or at the nickel-beta-beryllide interface; whereas for the beryllium-1% silver the fracture path is entirely within the beryllium-gamma-beryllide interface. The increase in silver from 1% to 8% or in the case of silver plated nickel (which is excessive silver) raises the beryllium-gamma-beryllide interface strength to above approximately 6000 p.s.i. making it stronger than the gamma-beryllide layer of the nickel-beta-beryllide interface.

#### Hardness

The hardness of gamma-nickel beryllide ( $Ni_3Be_{21}$ ) is about 1300 (diamond pyramid number) which compares quite favorably with alumina (1200). The two phase transition region ( $Ni_3Be_{21}$  + beryllium-silver) which lies between the very hard gamma-nickel beryllide and the beryllium has a hardness of 600. Representative micro-hardness values for a number of compounds applicable as coatings for beryllium are shown in Table I. The beryllium compounds listed in the table were formed at about 1100° C. For the beryllide it was found that the presence of silver does not affect hardness although its presence is a critical factor in achieving adherence. However, it appears that there is a critical temperature which must be achieved to obtain high hardness values in the beryllium compounds as those compounds formed at 1000° C. do not have a high hardness.

Table I.—Microhardness values

| Material:           | Hardness<br>(diamond pyramid No.) |    |
|---------------------|-----------------------------------|----|
| $Ni_3Be_{21}$ ----- | 1300                              | 70 |
| $Al_2O_3$ -----     | 1200                              |    |
| NiBe -----          | 675                               |    |
| Beryllium -----     | 165                               |    |
| Nickel -----        | 115                               |    |
| CrBe -----          | 1250                              | 75 |

#### Thickness

Relatively thick beryllide layers can be formed in a short time in accordance with this invention. For example, at 1100° C. with a beryllium-4% silver alloy an 0.030 inch layer is formed in about 3 hours. FIGURE 3 shows the total beryllide thickness formed for the various alloys as a function of diffusion time at 1000° C. to 1100° C. The thickness increases as would be expected with time and temperature. It is noted that silver content also has this effect which appears due to an indirect increase in temperature since this addition lowers the melting temperature of the alloy formed. Of course, the ultimate thickness of any particular coating is dependent on the particular use or application desired.

15 Although the invention has been shown and described in terms of particular embodiments, it will be appreciated that various changes and modifications are conceivable which do not depart from its spirit and scope. Maximum hardness is achieved with pure gamma-nickel beryllide, however, slight deviations from this stoichiometric relationship are deemed to be within the scope of this invention. Accordingly, such changes and modifications as are obvious to one skilled in the art are also deemed to be within the scope of the invention.

25 What is claimed is:

1. An article comprising: a beryllium body having thereon in adherent relationship a wear resistant coating composed of first and second regions, said first region comprising a two phase composition of a beryllium-silver alloy and gamma-nickel beryllide, said second region comprising gamma-nickel beryllide.

2. An article comprising: a body, the composition of which is at least substantially beryllium, having thereon in adherent relationship a wear resistant coating composed of first and second regions, said first region comprising a two phase composition of a beryllium-silver alloy and gamma-nickel beryllide, said second region comprising gamma-nickel beryllide.

3. An article comprising: a body, the composition of which is about 1% to about 8% silver, balance beryllium, said body having thereon in adherent relationship a wear resistant coating composed of first and second regions, said first region comprising a two phase composition of a beryllium-silver alloy and gamma-nickel beryllide, said second region comprising gamma-nickel beryllide.

4. The method of forming a beryllide coating on a beryllium body comprising the steps of:

(A) diffusion bonding a nickel body in the presence of silver to said beryllium body at a temperature of at least about 1075° C. for a time sufficient to form a diffusion couple consisting of discrete regions of nickel, beta-nickel beryllide, gamma-nickel beryllide, a two phase region of a beryllium-silver alloy plus gamma-nickel beryllide and a region of beryllium, and  
(B) removing said nickel and beta-nickel beryllide regions to expose said gamma-nickel beryllide region as an outer coating on said beryllium body.

5. The method of forming a beryllide coating on a beryllium body comprising the steps of:

(A) positioning said beryllium body in bonding relationship with a body of nickel,  
(B) inserting an amount of silver between said bodies,  
(C) heating said bodies in a vacuum to a temperature of at least about 1075° C. for at least 1/2 hour to form a diffusion couple therebetween consisting of discrete regions of nickel, beta-nickel beryllide, gamma-nickel beryllide, a two phase region of a beryllium-silver alloy plus gamma-nickel beryllide, and a beryllium region, and  
(D) removing said nickel and beta-nickel beryllide regions to expose said gamma-nickel beryllide region as an outer coating on said beryllium body.

6. The method of forming a beryllide coating on a beryllium body comprising the steps of:

- (A) contacting said beryllium body with a nickel body having a silver plate thereon,  
 (B) heating said bodies to a temperature of at least about 1075° C. for at least 1/2 hour to form a diffusion couple consisting of discrete regions of nickel, beta-nickel beryllide, gamma-nickel beryllide, a two phase region of a beryllium-silver alloy plus gamma-nickel beryllide, and a region of beryllium, and  
 (C) removing said nickel and beta-nickel beryllide region to expose said gamma-nickel beryllide as an outer coating bonded to said beryllium body by said two phase region.

7. The method of forming a gamma-nickel beryllide coating bonded to a body consisting substantially of beryllium by means of a two phase transition region comprising the steps of:

- (A) providing a body of a beryllium-silver alloy,  
 (B) contacting said body with a nickel body,  
 (C) heating said bodies at a temperature of at least about 1075° C. for at least 1/2 hour to form a diffusion couple consisting of discrete regions of nickel, beta-nickel beryllide, gamma-nickel beryllide, a two phase region of a beryllium-silver alloy plus gamma-nickel beryllide and said beryllium-silver alloy, and  
 (D) removing said nickel and beta-nickel beryllide regions to expose said gamma-nickel beryllide as an outer coating bonded to said beryllium-silver alloy by said two phase region.

8. The method of forming a gamma-nickel beryllide coating bonded to a beryllium-silver alloy body by a two phase transition region comprising the steps of:

- (A) providing a body of a beryllium-silver alloy containing from about 1% up to about 8% silver, balance beryllium,  
 (B) contacting said body with a nickel body,  
 (C) heating said bodies at a temperature of at least about 1070° C. for at least 1/2 hour to form a diffusion couple consisting of discrete regions of nickel, beta-nickel beryllide, gamma-nickel beryllide, a two phase region of a beryllium-silver alloy plus gamma-nickel beryllide and said beryllium-silver alloy and  
 (D) removing said nickel and beta-nickel beryllide regions to expose said gamma-nickel beryllide region as an outer coating bonded to said beryllium-silver alloy by said two phase region.

#### References Cited by the Examiner

##### UNITED STATES PATENTS

|           |        |                  |       |        |
|-----------|--------|------------------|-------|--------|
| 2,846,792 | 8/1958 | Walker et al.    | ----- | 29—194 |
| 2,969,309 | 1/1961 | Finniston et al. | ----- | 29—194 |
| 3,044,156 | 7/1962 | Whitfield et al. | ----- | 29—194 |
| 3,082,521 | 3/1963 | Cohen            | ----- | 75—150 |

DAVID L. RECK, *Primary Examiner.*

HYLAND BIZOT, *Examiner.*

R. O. DEAN, *Assistant Examiner.*